

# United States Patent

[11] 3,619,191

|                |                                                   |           |         |                    |         |
|----------------|---------------------------------------------------|-----------|---------|--------------------|---------|
| [72] Inventor  | Robert C. Desjarlais<br>South Hadley Falls, Mass. | 3,069,268 | 12/1962 | Herrick .....      | 96/75 X |
| [21] Appl. No. | 667,365                                           | 3,076,707 | 2/1963  | Lawton et al. .... | 96/75   |
| [22] Filed     | Sept. 13, 1967                                    | 3,052,542 | 9/1962  | Sulich.....        | 96/91 X |
| [45] Patented  | Nov. 9, 1971                                      | 3,113,025 | 12/1963 | Bialczak .....     | 96/49 X |
| [73] Assignee  | The Tecnifax Corporation<br>Holyoke, Mass.        | 3,248,220 | 4/1966  | Van Rhijn .....    | 96/91   |
|                |                                                   | 3,410,688 | 11/1968 | Welch .....        | 96/91   |

## FOREIGN PATENTS

|         |        |                    |       |
|---------|--------|--------------------|-------|
| 937,510 | 9/1963 | Great Britain..... | 96/91 |
|---------|--------|--------------------|-------|

## OTHER REFERENCES

Dinaburg, M. S., " Photosensitive Diazo Cpd's," 1964, pages 50-53.

Nollev, C. R., " Textbook of Organic Chemistry," 2nd Ed., 1958, page 341

Kosar, J., " Light-Sensitive Systems," 1965, pages 292-296.

*Primary Examiner*—Norman G. Torchin

*Assistant Examiner*—Charles L. Bowers, Jr.

*Attorneys*—William J. Foley, Stanton T. Hadley and John W. Kane, Jr.

## [54] DIAZO-TYPE MATERIALS 39 Claims, No Drawings

|                      |                                    |
|----------------------|------------------------------------|
| [52] U.S. Cl.        | 96/75,                             |
|                      | 96/49, 96/91                       |
| [51] Int. Cl.        | G03c 1/60,<br>G03c 1/58, G03c 1/54 |
| [50] Field of Search | 96/91, 75,<br>49                   |

## [56] References Cited

### UNITED STATES PATENTS

|           |         |                       |         |
|-----------|---------|-----------------------|---------|
| 1,803,906 | 5/1931  | Kreiger et al. ....   | 96/91   |
| 2,531,485 | 11/1950 | Van Giehn et al. .... | 96/91   |
| 2,617,726 | 11/1952 | Kessels.....          | 96/91 X |
| 2,661,291 | 12/1953 | Slifkin.....          | 96/91 X |
| 2,717,832 | 9/1955  | Sulich.....           | 96/91   |
| 2,893,866 | 7/1959  | Haefeli .....         | 96/91 X |

**ABSTRACT:** Light-sensitive diazo compositions containing light-sensitive diazonium derivatives of dialkoxy-substituted paraphenylenediamines, at least one coupling component for said diazonium derivatives, and at least one background discoloration inhibitor are disclosed.

## DIAZO-TYPE MATERIALS

## BACKGROUND OF THE INVENTION

## Field of the Invention

This invention relates to novel, light-sensitive diazotype materials of the two-component type which contain a diazonium derivative of a dialkoxy-substituted paraphenylenediamine as the diazo component, and which are less susceptible to background discoloration after development than are similar materials of the prior art. Certain diazo compositions within the scope of this invention are useful in preparing black-line prints which are highly resistant to light fading and which exhibit a neutral black-line development over a wide image-density range, as well as being resistant to background discoloration subsequent to their development.

## DESCRIPTION OF THE PRIOR ART

As is well-recognized by those skilled in the art, the two most widely accepted diazo processes are often referred to as the one-component process or the semi-wet development process, wherein the light-sensitive diazotype material contains the diazo compound in the absence of a coupler and the development step in said process consists of applying a developing solution containing a coupler to the diazotype material; and the two-component process or the "dry" development process, wherein the light-sensitive diazotype material contains both the diazo compound and the coupling component or components and wherein the development step in said process consists of exposing the diazotype material to an alkaline atmosphere, which is usually a mixture of ammonia and water vapors.

Although the two-component or dry development process has certain advantages over the one-component or semi-wet development process, (the major advantage being the one most obvious—the fact that it is essentially a dry process), there has, up until now, been certain serious disadvantages associated with the dry process also. In order to obtain certain desired colors in the developed print, it is necessary to use a relatively specific class of diazonium compounds in combination with a specific class or classes of coupling components; and, although these combinations may result in the color desired in the final print, this print oftentimes exhibits unacceptable background discoloration in the exposed areas wherein the diazo component has been decomposed. This is particularly true in those cases where the diazo component is a diazonium derivative of a dialkoxy-substituted p-phenylene diamine. Although diazonium derivatives of dialkoxy-substituted p-phenylene diamines are known to be useful as diazo components in diazotype materials, particularly in one-component diazotype materials, their use in two-component diazotype materials has been severely limited, due to the pronounced tendency of such materials to discolor after development in the background or "burnout" areas. Without wishing to be bound to any particular theory as to the cause of this background discoloration, it is believed that this discoloration is due to the subsequent oxidation of the photolysis products of these types of diazo components (i.e., the initially colorless derivatives of these diazo components which are formed in the background or nonimage areas upon exposure of the light-sensitive diazotype material to a light source of sufficient intensity and of the proper wavelength to effect "imaging" of the diazotype material), due to other components and/or impurities which are present in the diazo layer. Until now, this problem of background discoloration which has been observed with these types of diazo components has restricted their use in two-component diazotype materials, despite the fact that they are in most other respects very suitable for use in diazotype materials.

In addition, there is also a well-recognized need in the diazo art for a diazotype material which results upon development in a neutral-black-line print which is neutral black over a wide range of image densities. Although there are diazotypec

materials available which may result in a black-line print at a given image density, the color of the print may vary considerably from the desired black at higher or lower image densities. It is believed that this "two-toning" is due to a difference in the coupling activities of the various couplers employed to obtain a black-line print, and that if the various couplers are not carefully matched for coupling activity, the difference in coupling rates between or among the coupling components results in images other than neutral black, particularly in the lower image density areas. Another factor which makes the achievement of a neutral black-line image over a wide image density range most difficult is the fact that many resulting azo dyes produced upon coupling or development of many of the previously available diazotype materials are subject to a color-shift or a change in shade with a change in the pH of the diazotype print, resulting in a shift or change in the color of the resulting azo dye from the desired neutral black. It is apparent that in order to obtain a neutral black-line print over a wide image density, the coupling rates of the various couplers employed must be very carefully matched to obtain a mixture of azo dyes in the developed print which is neutral black over a wide range, and the resulting azo dyes must not be subject to a color-shift or change in shade with a change in pH. It is, of course, also highly desirable that the "burnout" or non-image areas of such a neutral black-line print exhibit little or no background discoloration upon aging. Until now, a two-component diazotype material with these desirable features was unavailable in the diazo art. As indicated above, although the diazonium derivatives of a dialkoxy-substituted p-phenylene diamines have heretofore been known to be capable of producing neutral black-line images over at least some ranges of image densities, their inherent tendency to discolor in the background or non-image areas has precluded their extensive use in a two-component diazotype material to form a black-line print.

## SUMMARY OF THE INVENTION

It has now been found that the incorporation of at least one background discoloration inhibitor into light-sensitive diazo compositions containing a diazonium derivative of a dialkoxy-substituted paraphenylenediamine as the diazo component substantially reduces the background discoloration which one normally obtains with diazo compositions wherein these types of diazo components are employed without such an inhibitor. As has been indicated above, derivatives of dialkoxy-substituted paraphenyl-enediamines have been found to be a potentially very useful class of diazo components, except for their tendency in developed prints to discolor in the background areas. It has been found that this class of diazo compounds is capable of producing azo dyes having excellent light fastness, bright shades, good resistance to color changes due to gas fading; and, with the proper choice of coupling components, dyes which form a neutral black image upon development. By incorporating a background discoloration inhibitor of the type hereinafter disclosed, two-component diazotype materials can be prepared using diazonium derivatives of dialkoxy-substituted p-phenylenediamines, said diazotype materials being essentially free from background discoloration after development.

## DESCRIPTION OF THE PREFERRED EMBODIMENTS

## The Diazo Component

As has hereinbefore been indicated, the light-sensitive compositions of this invention employ, as the diazo component, light-sensitive diazonium compounds derived from dialkoxy-substituted p-phenylenediamines. More particularly, these diazonium compounds are compounds formed from a p-phenylenediamine having a general formula selected from the group consisting of:



and



and

wherein R is an alkyl group or cycloalkyl group containing from about 1 to about 6 carbon atoms, R<sup>1</sup> and R<sup>2</sup> are alkyl groups containing from 1 to about 3 carbon atoms, and the group represented by



is a saturated, nitrogen-containing, heterocyclic ring, containing up to about 7 atoms in said ring. Diazonium derivatives of compounds wherein R is a branched alkyl group, such as isopropyl, isobutyl, secondary butyl, tertiary butyl, tertiary pentyl, 2-pentyl, 3-pentyl, and the like; or a cycloalkyl group such as cyclopentyl, cyclohexyl, and the like; and wherein the group represented by



is a morpholinyl group are preferred. The methods of preparing both the dialkoxy-substituted p-phenylene materials and their diazonium derivatives are well-known in the art and are described, for example, in U.S. Pat. No. 3,028,240, which relates to the use of these types of compounds in a single-component diazotype process. As is indicated in this patent, these diazo compounds are particularly useful in preparing black-line prints when they are employed with the proper coupling components in a one-component process. However, as has been indicated above, the use of these compounds in a two-component process has heretofore been limited, due to the fact that the resulting prints exhibited a pronounced degree of background discoloration.

The diazo component employed in the present invention is preferably employed in the form of a stabilized diazo salt, such as a metal halide salt, a sulfate salt, and the like. Illustrative of the types of diazonium compounds which may be employed in this invention are compounds such as 4-morpholino-2,5-di



and the like.

#### The Coupling Component

As appreciated by one skilled in the art, the choice of coupler or couplers depends primarily upon the color desired in 30 the resulting diazo print, and the speed required for development. Illustrative of the types of couplers which can be employed in preparing the diazotype materials of this invention are couplers such as resorcinol, 2-methyl resorcinol, 4-methyl resorcinol, 5-methyl resorcinol, 2-methyl 4-ethyl resorcinol, 2,4 dichloro resorcinol, 4,6 dichloro resorcinol, 4-chloro resorcinol, 4-bromo resorcinol, 4-iodo resorcinol, 4-fluoro resorcinol, N-β-hydroxy-ethyl-α-resorcylamide, α-resorcylamide, N-phenyl α-resorcylamide, resorcinol 5-sulfonic acid, resorcinol 4-sulfonic acid, α-resorcyl acid, resorcinol 4,6 disulfonic acid, resorcinol mono-methyl ether, resorcinol mono benzoate, resorcinol mono acetate, resorcinol mono formate, β-resorcyl acid methyl ester, β-resorcyl acid amide, β-resorcyl acid, α-naphthol β-naphthol 2,3 dihydroxy naphthalene, α-resorcyl acid, α-resorcyl acid methyl ester, α-resorcyl acid amide, 4 bromo-3,5-dihydroxybenzoic acid amide, 4-chloro-3,5-dihydroxybenzoic acid amide, bis-(2,4-dihydroxy phenyl sulfide), bis-(2,4-dihydroxy phenyl sulfoxide), condensation product of 5-amino resorcinol and 45 cyanuric chloride, hydroquinone monomethyl ether, phloroglucinol, phloroglucinol mono methyl ether, 1,3,5 trihydroxy-2-methyl benzene, O' hydroxy diphenyl, 3,3',5-trihydroxy diphenyl, 2,4,4'-trihydroxy diphenyl, 2,2',4,4'-tetrahydroxy diphenyl, 2,2',4,4'-tetrahydroxy 3,3'-dimethyl 5,5'-dichlorodiphenyl sulfide, 2,2', 4,4'-tetrahydroxy 5,5'-dichloro diphenyl sulfide, 2,3 dihydroxy naphthalene 6 sulfonic acid, 1 naphthol-2 sulfonic acid, 1 naphthol-3 sulfonic acid, 1 naphthol-4 sulfonic acid, 2 hydroxyl naphthalene-3,6 -disulfonic acid, 1,8 dihydroxy naphthalene-3,6 disulfonic acid, 1,8 dihydroxy naphthalene-3,5 disulfonic acid, 1,8 dihydroxy naphthalene-4 sulfonic acid, 1,8 dihydroxy naphthalene-3 sulfonic acid, 2,8 dihydroxy naphthalene-6 sulfonic acid, 3,8 dihydroxy naphthalene-6 sulfonic acid 8 acetylarnino-1 -naphthol-5-sulfonic acid, 2 hydroxy naphthalene-6-sulfonic acid, 2 hydroxy naphthalene-4-sulfonic acid, 2 hydroxy naphthalene-6,8-disulfonic acid, 2 hydroxy naphthalene-7-sulfonic acid, 1 hydroxy naphthalene-6,8-disulfonic acid, 2 hydroxy-3 naphthoic-(3'nitro) anilide, 2 hydroxy-3 naphthoic-(4'chloro) anilide, 2 hydroxy-3 naphthoic-(4'methoxy) anilide, 2 hydroxy-3 naphthoic-(2'methoxy) anilide, 2 hydroxy-3 naphthoic-(2' methyl) anilide, 2 hydroxy-3 naphthoic-(4' methyl) anilide, 2 hydroxy-3 naphthoic-(3'



(methyl) anilide, 2 hydroxy-3 naphthoic-(2',5' dimethoxy) anilide, 2 hydroxy-3 naphthoic-(1 naphthalanilide), 2 hydroxy-3 naphthoic-(2 naphthalanilide), 2 hydroxy-3 naphthoic-(2' methyl, 4' chloro) anilide, 2 hydroxy-3 naphthoic-(2' chloro) anilide, (acetoacetyl amino benzene), (acetoacetyl-benzylamide), (2 acetoacetylamino-1-methoxy benzene), (2 chloro-1-acetoacetylamino-benzene), (4-chloro-1-acetoacetylamino-benzene), (2,5-dichloro-1-acetoacetylamino-benzene), (4-acetoacetylamino-1,3-dimethoxy benzene), (6-acetoacetylamino-1,4-dimethoxy benzene), (6 chloro-4-acetoacetylamine-1,3-dimethoxy benzene), (1-acetoacetylamino-naphthalene), (4-acetoacetylamino-1-ethoxy-benzene), 1 phenyl-3-methyl-5-pyrazolone, 1 phenyl-5-pyrazolone-3-carboxylic amide, 1-(Benzene-2' sulfonic acid)-3-phenyl-5-pyrazolone, 1-(Benzene-3' sulfonic acid)-3-methyl-5-pyrazolone, 1-(Benzene-4' sulfonic acid)-3-methyl-5-pyrazolone, and the like.

Of particular interest for use as orange or sepia couplers N,N'-diaryl-substituted this invention are a class of substituted diresorcylic sulfide and sulfoxide compounds, i.e., compounds having the diazotype formula



wherein R<sup>4</sup> is hydrogen; an alkyl group containing from one to about six carbon atoms, such as methyl, ethyl, propyl, butyl, amyl, hexyl, 2-ethylbutyl, and the like; and unsubstituted aryl group or halo-substituted aryl group such as p-chlorophenyl, m-chlorophenyl, phenyl, and the like; an aralkyl group, including alkyl-substituted aralkyl groups and halo-substituted aralkyl groups, such as benzyl p-methylbenzyl, p-chlorobenzyl, o-chlorobenzyl and the like; an alkaryl group, including halo-substituted alkaryl groups, such as xylyl, chloroxylyl, tolyl, chlorotolyl, and the like; an alkoxy group containing from one to about six carbon atoms, such as methoxy, propoxy, butoxy, amyloxy, and the like; an aryloxy group including halo-substituted aryloxy groups such as phenoxy, p-chlorophenoxy and the like, an aralkoxy group including halo-substituted aralkoxy groups such as benzylxyloxy, p-chlorobenzylxyloxy, and the like; or a halogen, such as chlorine, bromine or iodine; Z is hydrogen or a halogen, such as chlorine, bromine or iodine, and wherein at least one of the groups represented by R<sup>4</sup> and Z is a group other than hydrogen. The substituted diresorcylic sulfides are particularly preferred.

The substituted diresorcylic sulfides described above are prepared by reacting sulfur dichloride in the presence of an inert solvent with a resorcinol substituted in the 2-position with an alkyl group, such as methyl group, an ethyl group, a propyl group, a butyl group, an amyl group, a 2-ethyl-butyl group, and the like; an aryl group or halo-substituted aryl group, such as a phenyl group, a p-chlorophenyl group, a m-chlorophenyl group, and the like; an aralkyl group, alkyl-substituted aralkyl group, or halo-substituted aralkyl group such as a benzyl group, a p-methylbenzyl group, a p-chlorobenzyl group, an o-chlorobenzyl group, and the like; and alkaryl group or halo-substituted alkaryl group, such as a xylyl group, a chloroxylyl group, a tolyl group, a chlorotolyl group, and the like; an alkoxy group, such as a methoxy group, a propoxy group, a butoxy group, an amyloxy group, and the like; an aryloxy group or halo-substituted aryloxy group, such as a phenoxy group, a p-chlorophenoxy group, and the like; an aralkoxy group or halo-substituted aralkoxy group, such as a benzylxyloxy group, a p-chlorobenzylxyloxy group, and the like; or a halogen, such as chlorine, bromine or iodine.

halo group, such as a chloro group, an iodo group, a bromo group, and the like; a resorcinol substituted in the 4-position with a halo group, such as a chloro group, an iodo group, a bromo group, and the like; or a resorcinol substituted in the 2-position with an alkyl group, such as a methyl group, an ethyl group, a propyl group, a butyl group, an amyl group, a 2-ethylbutyl group, and the like; an aryl group or halo-substituted aryl group, such as a phenyl group, a p-chlorophenyl group, a m-chlorophenyl group, and the like; an aralkyl group, alkyl-substituted aralkyl group, or halo-substituted aralkyl group such as a benzyl group, a p-methylbenzyl group, a p-chlorobenzyl group, an o-chlorobenzyl group, and the like; and alkaryl group or halo-substituted alkaryl group, such as a xylyl group, a chloroxylyl group, a tolyl group, a chlorotolyl group, and the like; an alkoxy group, such as a methoxy group, a propoxy group, a butoxy group, an amyloxy group, and the like; an aryloxy group or halo-substituted aryloxy group, such as a phenoxy group, a p-chlorophenoxy group, and the like; an aralkoxy group or halo-substituted aralkoxy group, such as a benzylxyloxy group, a p-chlorobenzylxyloxy group, and the like; and in the 4-position with a halo group, such as a chloro group, an iodo group, a bromo group, and the like. Inert solvents such as diethyl ether, dipropyl ether, ethyl acetate, and the like, can be employed, and the reaction temperature can vary, depending on the type of inert solvent which is employed. Temperatures of from about 5° C. to about 35° C. are preferred, with temperatures of from about 5° to about 15° C. being particularly preferred with the lower-boiling inert solvents. It is also preferred to conduct the reaction under an atmosphere of a dry, inert gas, such as nitrogen, helium, and the like, said gas being used to facilitate the removal of the hydrogen chloride which is evolved. The resulting substituted diresorcylic sulfides compounds are easily recovered as crystalline solids having relatively high melting points (in excess of 150° C.) and are readily purified by recrystallization from alcohols or ketones, such as acetone and methylethyl ketone. The sulfoxide derivatives of these substituted diresorcylic sulfides are prepared by treating the sulfide with an oxidizing agent, such as hydrogen peroxide, chromic oxide, potassium permanganate, and the like. Illustrative of the types of compounds within this preferred class of orange or sepia couplers are compounds such as 4,4'-tetrahydroxy-3,3'-dimethyldiphenyl sulfide, 4,4'-tetrahydroxy-5,5'-dichlorodiphenyl sulfide, 4,4'-tetrahydroxy-3,3'-dimethyl-5,5-dichlorodiphenyl sulfide, 4,4'-tetrahydroxy-3,3'-dimethyldiphenyl sulfoxide, and the like. It is believed that the diresorcylic sulfides and sulfoxides which are substituted in both the 3,3' positions and the 5,5' positions are novel compositions of matter, and they are claimed as such herein. Quite unexpectedly, they have been found to be excellent yellow shading components for diazo compositions, and they exhibit coupling rates which are highly compatible with the coupling rates of the blue couplers which are usually employed.

The following preparations are provided to illustrate more specifically the methods of preparing the preferred orange or sepia couplers for use in the present invention.

#### 60 A. PREPARATION OF 4,4'-TETRAHYDROXY-3,3'-DIMETHYL DIPHENYL SULFIDE

18.7 grams of 2-methyl resorcinol were dissolved with stirring in 48 ml. of ethyl acetate. A solution of 7.8 grams of sulfur dichloride in 58 ml. ethyl acetate was then added slowly to the 2-methyl resorcinol-ethyl acetate solution, and the reaction mixture was stirred at room temperature for one-half hour, with dry nitrogen being introduced into the reaction flask to remove the hydrogen chloride which evolves from the reaction. The reaction mixture was then washed with water, separated, and the ethyl acetate fraction was vacuum distilled. The remaining light-yellow solid reaction product was slurried in warm toluene, filtered and dried to yield 7.5 grams (36 percent of theoretical) of a product which was insoluble in cold water, toluene and benzene and soluble in alcohols and



and the like; carbamyl groups, including N-substituted carbamyl groups, for example, a methylcarbamyl group



a benzylcarbamyl group



a morpholinocarbamyl group



and the like;  
and acyl groups, for example, an acetyl group



a propionyl group



a butyryl group



a benzoyl group



and the like. Compounds wherein X is a trifluoromethyl group, an unsubstituted sulfamyl group, or an aliphatic acyl group, such as an acetyl group are particularly preferred. Those 3'-substituted 2-hydroxy, 3-naphthalimides wherein the non-chromophoric and electron-withdrawing substituent represented by X contains a sulfonyl group or carbonyl group attached directly to the aniline nucleus are believed to be novel compositions of matter, and are claimed as such in a separate application filed on even date as the present application, U.S. Serial No. 667,372.

The preferred 3'-substituted, 2-hydroxy, 3-naphthalimides described above can be prepared either by reacting a meta-substituted aniline having the formula



wherein X is as hereinbefore defined with 2-hydroxy, 3-naphthoyl chloride in the presence of a suitable solvent, or by reacting such a meta-substituted aniline with 2-hydroxy-3-naphthoic acid in the presence of an inert solvent and phosphorus trichloride. Illustrative of the meta-substituted anilines which can be employed in preparing these preferred blue couplers are compounds

such as m-(trifluoromethyl) aniline



methyl m-aminobenzoate



ethyl m-aminobenzoate



propyl m-aminobenzoate



butyl m-aminobenzoate



m-aminobenzenesulfonamide



N-methyl-m-aminobenzenesulfonamide



N-benzyl-m-aminobenzenesulfonamide



N-allyl-m-aminobenzenesulfonamide



N-morpholinopropyl-m-aminobenzene-sulfonamide



m-aminobenzamide



N-methyl-m-aminobenzamide



N-benzyl-m-aminobenzamide



m-aminobenzmorpholide

11



m-aminoacetophenone



ethyl-m-aminophenyl ketone



propyl-m-aminophenyl ketone



phenyl-m-aminophenyl ketone



and the like.

When the preferred 3'-substituted, 2-hydroxy, 3-naphthalenides are prepared by reacting a meta-substituted aniline with 2-hydroxy, 3-naphthoyl chloride, the meta-substituted aniline is first dissolved in a solvent such as toluene, dioxane, methylene chloride, pyridine, and the like, and then 2-hydroxy, 3-naphthoyl chloride is added to the aniline solution. The resulting reaction mixture is stirred overnight, and then the desired 3'-substituted, 2-hydroxy, 3-naphthalenide reaction product is isolated in the usual manner. The reaction between the meta-substituted aniline and 2-hydroxy, 3-naphthoyl chloride can be accelerated by refluxing the reaction mixture, and the yield of the desired 3'-substituted, 2-hydroxy, 3-naphthalenide can be improved by incorporating an acid acceptor in the said reaction mixture. In many instances the solvent used to dissolve the meta-substituted aniline reactant can also serve as an acid acceptor (e.g., solvents such as pyridine, picoline, triethylamine, and the like), or the m-substituted aniline can itself serve as an acid acceptor, if it is employed in amounts in excess of the theoretical amount necessary to react with all of the 2-hydroxy, 3-naphthoyl chloride present in the reaction mixture.

When the preferred 3'-substituted, 2-hydroxy, 3-naphthalenides are prepared by reacting a meta-substituted aniline with 2-hydroxy, 3-naphthoic acid in the presence of an inert solvent and phosphorus trichloride, 2-hydroxy, 3-naphthoic acid and the m-substituted aniline are first dissolved or slurried in a relatively inert solvent such as toluene, methylene chloride, dichloroethane, and the like; and then phosphorus trichloride is added at a controlled rate in order to prevent the temperature of the reaction mixture from exceeding about 55° C. Upon completion of the addition of the phosphorus trichloride the reaction mixture is then refluxed until substantially all of the hydrochloric acid formed from the reaction is driven off. The desired 3'-substituted, 2-hydroxy, 3-naphthalenide reaction product can be isolated from the reaction mixture by direct filtration if it has precipitated from solution during the course of the reaction; otherwise it can be isolated by cooling, or by the addition of solvents in which the desired product is known to be insoluble.

12

Illustrative preparations of the preferred 3'-substituted, 2-hydroxy, 3-naphthalenides are as follows:

5 A. PREPARATION OF 2-HYDROXY, 3-NAPHTHOIC ACID,

3'-(SULFONAMIDO) ANILIDE



15 15 BY REACTING m-AMINOBENZENESULFONAMIDE WITH

2-HYDROXY, 3-NAPHTHOYL CHLORIDE

20 17.2 grams of m-aminobenzenesulfonamide were dissolved in 100 ml. of dry pyridine. 20.6 grams of 2-hydroxy, 3-naphthoyl chloride which was prepared by refluxing 2-hydroxy, 3-naphthoic acid and thionyl chloride in methylene chloride, were then added to the aminobenzenesulfonamide-pyridine solution. Upon completion of the addition of naphthoyl chloride to the aminobenzenesulfonamide-pyridine solution, the resulting reaction mixture was refluxed for 2 hours at 118° C. The reaction mixture was then cooled to room temperature and 500 ml. of water were added. The 2-hydroxy, 3-naphthoic acid, 3'-(sulfonamido) anilide reaction product precipitated in the form of a cream colored solid. After filtering, the solids were washed with water, slurried in isopropanol, and then re-filtered. The yield was 21.5 grams of a white solid having a melting point of 276° to 280° C. Carbon-35 hydrogen-nitrogen analysis of the product was as follows:

|    | Found    | Theoretical |
|----|----------|-------------|
| 40 | Hydrogen | 4.3340%     |
|    | Nitrogen | 8.20%       |
|    | Carbon   | 59.60%      |

Infrared analysis was as follows:

45 Strong amide absorption bands at 6.0 and 6.5 microns.  
Strong sulfonamide absorption bands at 6.98, 7.55 and 8.67 microns.  
Medium-NH<sub>2</sub> and



50 absorption bands at 3.0 microns.

55 Weak-NH<sub>2</sub> bands absorption at 3.1 microns.

B. PREPARATION OF 2-HYDROXY, 3-NAPHTHOIC ACID

3'-(TRIFLUOROMETHYL)ANILIDE



60 BY REACTING 2-HYDROXYL, 3-NAPHTHOIC ACID WITH m-(TRIFLUOROMETHYL)ANILINE IN THE

65 PRESENCE OF PHOSPHORUS TRICHLORIDE

70 5.6 grams of phosphorus trichloride were added slowly while stirring, to a slurry of 18.8 grams (0.1 mole) of 2-hydroxy, 3-naphthoic acid and 12.3 grams (0.1 mole) of m-trifluoromethyl)aniline in 190 ml. of anhydrous toluene. The 75 temperature of the reaction mixture rose to 45° C. and stirring became difficult. The reaction mixture was then refluxed until

substantially all of the hydrochloric acid formed in the reaction was driven off. The remaining reaction mixture was then poured into a beaker and cooled, and the solid 2-hydroxy, 3-naphthoic acid 3'-(trifluoromethyl)anilide reaction product was collected by filtration. The solid reaction product was air-dried, slurried in 5 percent aqueous  $\text{KHCO}_3$ , filtered, and washed well with water. The solids were then stirred in hot isopropanol and refiltered to yield 17 grams of a white solid product having a melting point of 234° to 235° C. Carbon-Hydrogen-Nitrogen analysis of the product was as follows:

|          | Found  | Theoretical |
|----------|--------|-------------|
| Hydrogen | 3.39%  | 3.64%       |
| Nitrogen | 3.49%  | 4.24%       |
| Carbon   | 64.57% | 65.10%      |

Infrared analysis was as follows:

Amide absorption bands at 7.60 and 14.35 microns.  
Trifluoromethyl absorption bands at 7.50, 8.54 and 8.90 microns.



absorption band at 3.05 microns.

Strong—OH absorption band at 3.23 microns.

Other preferred 3'-substituted, 2-hydroxy, 3-naphthanilide couplers which can be prepared in a manner similar to the preparations set forth above are compounds such as 2-hydroxy, 3-naphthoic acid, 3'-(acetyl)anilide



2-hydroxy, 3-naphthoic acid, 3'-(N-allylsulfonamido) anilide



2-hydroxy, 3-naphthoic acid, 3'-(N-benzylsulfonamido) anilide



2-hydroxy, 3-naphthoic acid, 3'-(N-morpholinopropylsulfonamido) anilide



2-hydroxy, 3-naphthoic acid, 3'-(N-methylsulfonamido) anilide



and the like.

The background discoloration inhibitors which have been found to be useful in preventing discoloration in the "burn-out" or background areas of the developed diazotype materials of this invention are N,N'Diaryl-substituted alkylene diamines, including N,N' methylene bridge tertiary amino derivatives thereof. These inhibitors have a general formula selected from the class consisting

10



and

15



20

wherein Ar is a group selected from the class consisting of a phenyl group and a hydrocarbyl-substituted phenyl group wherein said hydrocarbyl substituents are in either the meta or para position; R5 is a divalent hydrocarbon radical having a chain of either two to three carbon atoms separating the nitrogen atoms of the diamine; R6 is a group selected from the class consisting of hydrogen, alkyl groups containing from one to five carbon atoms, aralkyl groups containing from seven to about 10 carbon atoms, and groups represented by Ar; and R7 is selected from the class consisting of a methylene group and hydrocarbyl-substituted methylene groups. Compounds wherein Ar is a phenyl group, m-tolyl group or p-tolyl group; R5 is an ethylene group, a methyl-substituted ethylene group, a 1,2-dimethyl-substituted ethylene group or an ethyl-substituted ethylene group, a phenyl-substituted ethylene group; R6 is hydrogen; and R7 is a methylene group or a phenyl-substituted methylene group are preferred. Illustrative of such compounds are compounds such as N,N'-diphenylethylenediamine

30



N,N'-di(m-tolyl) ethylene diamine

35



N,N'-di(p-tolyl) ethylene diamine

40



N,N'-diphenyl-1,2-propylenediamine

45



N,N'-diphenyl, 2,3-butylenediamine

50



N,N'-diphenyl, 1,2-butylenediamine

55



N,N'-diphenylstyrenediamine

60



1,2,3-triphenylimidazolidine

15



1,3-di(m-tolyl)-2-phenylimidazolidine



1,3-di(p-tolyl)-2-phenylimidazolidine



1,2,3-triphenyl, 4-methylimidazolidine



1,2,3-triphenyl, 4,5 dimethylimidazolidine



1,2,3-triphenyl, 4-ethylimidazolidine



1,2,3,4-tetraphenylimidazolidine



and the like.

16

Although the amount of inhibitor which is employed in a coating composition has not been found to be narrowly critical from about 0.10 part by weight of inhibitor per 100 parts by volume of the coating mixture to about 2.0 parts by weight

5 of inhibitor per 100 parts by volume of the coating mixture is preferred, with about from 0.25 part by weight to about 1.0 part by weight being particularly preferred. Mixtures of these background discoloration inhibitors may also be employed, as well as mixtures of these types of inhibitors with other types of

10 inhibitors or antioxidants.

Inhibitors having the general formula:



20 wherein Ar, R<sup>5</sup> and R<sup>6</sup> are as hereinbefore defined can be prepared by reacting an aromatic amine such as aniline, para-toluidine, meta-toluidine, and the like, with a dihalo-substituted alkane or aralkane, such as ethylene dichloride; 1,2, dibromobutane; 2,3 dibromobutane; 1,2 dibromopropane; 25 styrene dibromide and the like. This reaction is a known reaction (cf., for example, Bennett, G.M. "Journal of the Chemical Society" 1919, 115, 577), and can be illustrated by the general equation:



35 wherein Ar, R<sup>5</sup> and R<sup>6</sup> are as hereinbefore defined and X represents a halogen, such as bromine, chlorine, and the like. The reaction is more specifically illustrated by the following preparation:

40 PREPARATION OF N,N'DI-(p-TOYL) ETHYLENE DIAMINE

42.8 Grams of para-toluidine,



45 50 (0.4 mole) were added to 9.9 grams of ethylene dichloride, C<sub>2</sub>-CH<sub>2</sub>-CH<sub>2</sub>-Cl, (0.1 mole); and the mixture was heated to reflux with stirring. At 135° C. a heavy precipitate began to form, and the mixture reached reflux temperature at 150° C. 55 After refluxing at 150° C. for 2 hours, the mixture was cooled to room temperature, at which temperature the reaction mixture was a solid. The solid reaction mass was then stirred with 200 ml. of water and filtered. A brownish-yellow solid was recovered and recrystallized from hexane to yield 13 grams of 60 a white solid which melted at 89° to 92° C. The N,N'di(p-tolyl)ethylenediamine product had the following carbon-hydrogen-nitrogen analysis:

| 65 | Found    | Theoretical |
|----|----------|-------------|
|    | Nitrogen | 11.63.66    |
|    | Carbon   | 80.25       |
|    | Hydrogen | 8.30        |

70 75 The infrared analysis of the N,N'-di-(p-tolyl)ethylenediamine product was as follows:  
Strong



secondary amine absorption band at 2.95 microns.  
Strong



absorption band at 6.56 microns.

Very Strong-CH<sub>2</sub>-absorption band at 6.85 microns.

Para-substituted doublet absorption bands at 12.34 microns and 12.42 microns.

Inhibitors having the general formula



wherein Ar, R<sup>5</sup> and R<sup>7</sup> are as hereinbefore defined can be prepared by reacting an aldehyde of the formula R<sup>8</sup>CHO wherein R<sup>8</sup> is a hydrocarbyl group with an N,N'-diaryl-substituted alkylene diamine of the general formula:



Wherein Ar and R<sup>5</sup> are as hereinbefore defined. For example, as disclosed by Moos in Berichte Der Deutschen Chemischen Gesellschaft, Vol. 20, page 732, 1,2,3-triphenylimidazolidine can be prepared by heating benzaldehyde with N,N-diphenylethylenediamine to boiling temperatures. The resulting imidazole derivative can be purified by recrystallization from alcohol, petroleum ether, benzene or other suitable solvents. Inhibitors such as 1,3-di(m-tolyl)-2-phenylimidazolidine and 1,3-di(p-tolyl)-2-phenylimidazolidine can be prepared in an analogous manner by substituting N,N'-di(m-tolyl)ethylenediamine and N,N'-di(p-tolyl)ethylenediamine for N,N'-diphenylethylenediamine in the procedure set forth above. A general equation for the reaction is as follows:



wherein Ar, R<sup>5</sup> and R<sup>8</sup> are as hereinbefore defined and the divalent group



is equivalent to the group R<sup>7</sup> as hereinbefore defined. The reaction is more specifically illustrated by the following preparation:

#### PREPARATION OF 1,2,3,-TRIPHENYLIMIDAZOLIDENE

21.2 Grams of diphenylethylenediamine,



(0.1 mole) in 100 ml. of toluene were slowly added to benzaldehyde. The resulting mixture was brought to reflux, and the water formed from the reaction was taken off and collected. When 1.8 ml. of water (0.1 mole) was collected, the reaction mixture was cooled, and the 1,2,3 triphenylimidazolidine product separated from solution. The solid reaction product was slurried in ethanol, filtered and air dried. 14.0 Grams of 1,2,3-triphenylimidazolidine were recovered, and the product had a melting point of 128° to 131° C. The carbon-hydrogen-nitrogen analysis of the product was as follows:

|          | Found | Theoretical |
|----------|-------|-------------|
| Nitrogen | 9.38  | 9.33        |
| Carbon   | 83.71 | 84.0        |
| Hydrogen | 6.84  | 6.66        |

The infrared analysis of the product was as follows:  
No.



absorption bands.

Strong phenyl ring absorption band at 6.25 microns.

Very Strong phenyl ring absorption band at 6.64 microns.

The light-sensitive diazo compositions of this invention can also contain any of the additional components which are often employed in such compositions, such as stabilizers for the diazo compound present in said compositions. The diazo composition is usually applied to a suitable base support in the form of a solution of various components in a solvent or solvents, which is then dried to form a coated support material which can be imaged and developed in the well-known manner of the diazotype art. The support may be any of the well-known support materials employed for diazo compositions, such as paper, cloth, transparentized paper, cellulose ester and ether films and polyester films having a subcoat thereon, such as mylar film having a subcoat of cellulose acetate butyrate.

The diazo coating compositions of this invention can be used to prepare light-sensitive diazotype materials, which are new and useful products for use in the fields of engineering drawing reproduction, microfilm visual communications and the graphic arts.

The following examples will serve to further illustrate this invention, but they are not intended to limit the scope thereof in any way.

#### EXAMPLE 1

A light-sensitive coating formulation was prepared containing the following components:

|    | COMPONENT                                                          | AMOUNT<br>g. |
|----|--------------------------------------------------------------------|--------------|
| 40 | Methanol                                                           | 52 cc.       |
|    | Acetone                                                            | 38 cc.       |
|    | Methyl ethyl ketone                                                | 10 cc.       |
|    | Hexafluorophosphoric Acid                                          | 0.6 cc.      |
|    | Thiourea                                                           | 0.3 g.       |
| 45 | 2,2',4,4'-Tetrahydroxy-3,3'-dimethyl diphenyl sulfide              | 0.75 g.      |
|    | 2-Hydroxy-3-naphthoic acid (3'-acetyl) anilide                     | 0.99 g.      |
|    | 2,2',4,4'-Tetrahydroxy-5,5'-dichloro-diphenyl sulfide              | 0.165 g.     |
|    | 1,2,3-Triphenylimidazolidine                                       | 0.75 g.      |
| 50 | 4 Morpholino-2,5-diisopropoxybenzene diazonium hexafluorophosphate | 2.3 g.       |

This coating formulation was coated onto a clear, cellulose diacetate base and dried. The dried, light-sensitive film was then exposed under a mercury vapor lamp light-source in a diazo duplicating machine using a silver halide master. The exposed film was then developed with ammonia vapor. A neutral black print over a wide range of image densities was obtained, and the resulting print exhibited excellent light-fade resistance and aging characteristics. Similar results are obtained when compounds such as N,N'-diphenylethylenediamine, N,N'-di(p-tolyl)ethylenediamine, N,N-di(m-tolyl) ethylene diamine, 1,3-di(p-tolyl)-2-phenylimidazolidine imidazolidine and 1,3-di(m-tolyl)-2-phenylimidazolidene are substituted for 1,2,3-triphenylimidazolidine in the formulation set forth above. However, if the N,N'-diaryl-substituted alkylene diamine background inhibitors are omitted from the formulation set forth above, an objectionable, reddish background appears in the background or "burn-out" areas of the developed print upon aging of the print. The amount of background discoloration which was observed with the above formulations was measured with a photovolt brightness meter, using White Cararra glass as the brightness standard. The background discoloration due to natural aging of the films prepared from the above formulations was as follows:

| Formulations (identified by inhibitor)                          | Initial brightness | After 5 months |
|-----------------------------------------------------------------|--------------------|----------------|
| 1,2,3-triphenylimidazolidine                                    | 75.0               | 72.5           |
| N,N'-dimethylethylene diamine                                   | 75.0               | 73.0           |
| N,N'-di(p-tolyl)ethylene diamine                                | 75.0               | 74.0           |
| N,N'-di(m-tolyl)ethylene diamine                                | 75.0               | 73.0           |
| 1,3-di(p-tolyl)-2-phenylimidazolidine                           | 75.5               | 73.5           |
| 1,3-di(m-tolyl)-2-phenylimidazolidine                           | 75.0               | 72.5           |
| Control (no N,N'-diaryl-substituted alkylene diamine inhibitor) | 75.5               | 161.0          |

1 With red discoloration observed.

The results set forth above clearly indicate that the N,N'-diaryl-substituted alkylene diamine inhibitors substantially reduce the amount of background discoloration which is normally obtained with two-component diazo-type materials wherein a diazonium derivative of a dialkoxy-substituted paraphenylenediamine is employed as the diazo component.

### EXAMPLE 2

A light-sensitive coating formulation was prepared containing the following components:

| COMPONENT                                                          | AMOUNT   |
|--------------------------------------------------------------------|----------|
| Methanol                                                           | 52 cc.   |
| Acetone                                                            | 38 cc.   |
| Methyl ethyl ketone                                                | 10 cc.   |
| Hexafluorophosphoric acid                                          | 0.6 g.   |
| Thiourea                                                           | 0.3 g.   |
| 2,2',4,4'-Tetrahydroxy-3,3'-dimethyl diphenyl sulfide              | 0.56 g.  |
| 2 Hydroxy-3-naphthoic acid (3'-sulfonamido) anilide                | 0.89 g.  |
| 2 Hydroxy-3-naphthoic acid (3'-(N-methylsulfonamido) anilide       | 0.15 gm. |
| 2,2'-Tetrahydroxy-5,5'-dichlorodiphenyl sulfide                    | 0.15 g.  |
| 1,2,3 Triphenylimidazolidine                                       | 0.75 g.  |
| 4 Morpholino-2,5-diisopropoxybenzene diazonium hexafluorophosphate | 2.3 g.   |

This coating formulation was coated onto a clear cellulose diacetate film base and dried. The dried, light-sensitive film was then exposed and developed in a manner similar to that set forth in example 1. A neutral black print was obtained from this film over a wide range of image densities, and the resulting print exhibited excellent light-fade resistance and aging characteristics.

### EXAMPLE 3

A light-sensitive coating formulation was prepared containing the following components:

| COMPONENT                                                          | AMOUNT  |
|--------------------------------------------------------------------|---------|
| Methanol                                                           | 52 cc.  |
| Acetone                                                            | 38 cc.  |
| Methyl ethyl ketone                                                | 10 cc.  |
| Hexafluorophosphoric acid                                          | 0.6 cc. |
| Thiourea                                                           | 0.6 g.  |
| 2 Hydroxy-3-naphthoic acid (3'acetyl)anilide                       | 0.99 g. |
| 2,2',4,4'-Tetrahydroxy-3,3'-dimethyl diphenyl sulfide              | 0.75 g. |
| 1,2,3 triphenylimidazolidine 0.75 g.                               |         |
| 4 Morpholino-2,5-diisopropoxybenzene diazonium hexafluorophosphate | 2.3 g.  |

This coating formulation was coated onto a clear, cellulose diacetate film base and dried. The dried, light-sensitive film was then exposed and developed in a manner similar to that set forth in example 1. A neutral black print was obtained from this film over a wide range of image densities, and the resulting print exhibited excellent light-fade resistance and aging characteristics. When the 2,2',4,4'-tetrahydroxy-3,3'-dimethyl diphenyl sulfide coupler is replaced with either 2,2',4,4'3,3'-dimethyl diphenyl sulfoxide or 2,2',4,4'3,3'-dimethyl 5,5'-dichlorodiphenyl sulfide in the above formulation, similar results are obtained, in that an excellent black print from the film is obtained over a wide range of image densities, and said print is resistant to subsequent background discoloration in the "burn-out" areas.

Similarly, when the 4-morpholino-2,5-diisopropoxybenzene diazonium hexafluorophosphate is replaced with either 4-morpholino-2,5-dicyclopropoxybenzene diazonium hexafluorophosphate or 4-morpholino-2,5-di(secondary-butoxy) benzene diazonium hexafluorophosphate in the above formulation, the desirable properties are also observed in the prints resulting from films prepared from said formulations. When the 2,2',4,4'-tetrahydroxy-3,3'-dimethyl diphenyl sulfide coupler in the above formulation is replaced with diresorcylic sulfide, diresorcylic sulfoxide or diresorcinol, the prints resulting from the films prepared from these formulations are also resistant to background discoloration, but blue, violet, or blue-black prints having reddish violet hues are obtained, rather than the neutral blacks which are obtained from formulations containing the preferred orange or sepia couplers.

We claim:

1. A light-sensitive diazo composition which comprises:  
A. at least one light-sensitive 2,5-dialkoxy-4-aminobenzene diazonium compound [derived from a dialkoxy-substituted-p-phenylene diamine] having the general formula selected from the class consisting of:

25 (1)



30 and

(2)



35

wherein Y is an inorganic acid anion; R is an alkyl group or a cycloalkyl group containing five or six carbon atoms; R<sup>1</sup> and R<sup>2</sup> are alkyl groups containing from one to three carbon atoms, and the group represented by



45 is a saturated, nitrogen-containing, heterocyclic ring containing six atoms in said ring;

- B. at least one azo coupling component for said diazonium compound;
- C. at least one background discoloration inhibitor having a general formula selected from the class consisting of:

55



60 wherein Ar is a phenyl group or an alkyl-substituted phenyl group wherein said alkyl substituents are in either the meta or para position, R<sup>5</sup> is a divalent hydrocarbon radical having a chain of two or three carbon atoms separating the nitrogen atoms in said inhibitor, wherein R<sup>6</sup> is a hydrogen atom, an alkyl group containing from one to five carbon atoms, an aralkyl group containing from seven to 10 carbon atoms.

2. A light-sensitive diazo composition as claimed in claim 1  
70 wherein the light-sensitive diazonium compound is [derived from 4-morpholino-2,5-diisopropoxyaniline, 4-morpholino-2,5-di(tertiary butoxy) aniline; 4-morpholino-2,5-di(secondary butoxy) aniline; or 4-morpholino-2,5-dicyclopropoxyaniline] a 4-morpholino-2,5-di(isopropoxy) benzene diazonium salt, a 4-morpholino-2,5-di(tertiary butoxy) benzene

diazonium salt, a 4-morpholino-2,5-di(secondary butoxy) benzene diazonium salt or a 4-morpholino-2,5-di(cyclopentox) benzene diazonium salt.

3. A light-sensitive diazo composition as claimed in claim 2 which comprises as a background discoloration inhibitor at least one compound selected from the class consisting of N,N'-diphenylethylenediamine, N,N'di(m-tolyl) ethylene diamine, N,N'di(p-tolyl) ethylenediamine, N,N'diphenylpropylenediamine, N,N'diphenyl-2,3-butlenediamine, N,N'-diphenyl-1,2-butlenediamine, N,N'-diphenylstyrenediamine, 1,2,3-triphenylimidazolidene, 1,3-di-(m-tolyl)-2-phenylimidazolidene, and 1,3-di(p-tolyl)-2-phenylimidazolidene, 1,2,3-triphenyl-4-methylimidazolidene, 1,2,3-triphenyl-4,5-dimethylimidazolidine, 1,2,3-triphenyl-4-ethylimidazolidine, and 1,2,3,4-tetraphenylimidazolidine.

4. A light-sensitive diazo composition as claimed in claim 3, wherein at least one of the compound is a compound having the general formula selected from the class consisting of:



wherein R<sup>4</sup> is selected from the class consisting of hydrogen alkyl groups containing from one to six carbon atoms, unsubstituted aryl groups, halo-substituted aryl groups; unsubstituted aralkyl groups, aralkyl groups having alkyl substituents on the aryl portion thereof, aralkyl groups having halo substituents on the aryl portion thereof, unsubstituted alkaryl groups, alkaryl groups having halo substituents on the alkyl portion thereof, alkoxy groups containing from one to six carbon atoms, unsubstituted aryloxy groups, halo-substituted aryloxy groups, unsubstituted aralkoxy groups, aralkoxy groups having halo substituents on the aryl portion thereof, and halogen atoms; Z is selected from the class consisting of hydrogen and halogen atoms; and wherein at least one of the groups represented by R<sup>4</sup> and Z is a group other than hydrogen.

5. A light-sensitive diazo composition as claimed in claim 4 wherein R<sup>4</sup> is methyl.

6. A light-sensitive diazo composition as claimed in claim 3 wherein at least one of the coupling components for the diazonium compound is a compound having the general formula:



wherein X is a non-chromophoric, electron-withdrawing substituent and is selected from the class consisting of trifluoromethyl groups, carbalkoxy groups, the sulfamyl group, N-substituted sulfamyl groups, the carbamyl group, N-substituted carbamyl groups and acyl groups.

7. A light-sensitive diazo composition as claimed in claim 3 wherein the coupling component for the diazonium compound is a mixture of A) a compound having the general formula selected from the class consisting of:



wherein R<sup>4</sup> is selected from the class consisting of hydrogen, alkyl groups containing from one to six carbon atoms, unsubstituted aryl groups, halo-substituted aryl groups; unsubstituted aralkyl groups, aralkyl groups having alkyl substituents on the aryl portion thereof, aralkyl groups having halo substituents on the aryl portion thereof, unsubstituted alkaryl groups, alkaryl groups having halo substituents on the alkyl portion thereof, alkoxy groups containing from one to six carbon atoms, unsubstituted aryloxy groups, halo-substituted aryloxy groups, unsubstituted aralkoxy groups, aralkoxy groups having halo substituents on the aryl portion thereof, and halogen atoms; Z is selected from the class consisting of hydrogen and halogen atoms; and wherein at least one of the groups represented by R<sup>4</sup> and Z is a group other than hydrogen and B) a compound having the general formula:



30 wherein X is a non-chromophoric, electron-withdrawing substituent and is selected from the class consisting of trifluoromethyl groups, carbalkoxy groups, the sulfamyl group, N-substituted sulfamyl groups, the carbamyl group, N-substituted carbamyl groups and acyl groups.

35 8. A light-sensitive diazo composition as claimed in claim 7, wherein the light-sensitive diazonium compound is 4-morpholino-2,5-diisopropoxybenzenediazonium hexafluorophosphate; the coupling components are 2,2',4,4'-tetrahydroxy-3,3'-dimethylidiphenyl sulfide, 2,2',4,4'-tetrahydroxy-5,5'-dichlorodiphenyl sulfide, and 2-hydroxy-3-naphthoic acid-(3'-acetyl)anilide; and the background discoloration inhibitor is 1,2,3-triphenylimidazolidine.

9. A light-sensitive diazo composition as claimed in claim 7, wherein the light-sensitive diazonium compound is 4-morpholino-2,5-diisopropoxybenzenediazonium hexafluorophosphate; the coupling components are 2,2',4,4'-tetrahydroxy-3,3'-dimethylidiphenyl sulfide, 2,2',4,4'-tetrahydroxy-5,5'-dichlorodiphenyl sulfide, and 2-hydroxy-3-naphthoic acid-(3'-acetyl)anilide; and the background discoloration inhibitor is N,N'-di(p-tolyl)ethylene diamine.

10. A light-sensitive diazo composition as claimed in claim 7, wherein the light-sensitive diazonium compound is 4-morpholino-2,5-diisopropoxybenzenediazonium hexafluorophosphate; the coupling compounds are 2,2',4,4'-tetrahydroxy-3,3'-dimethylidiphenyl sulfide, 2,2',4,4'-tetrahydroxy-5,5'-dichlorodiphenyl sulfide, and 2-hydroxy-3-naphthoic acid-(3'-acetyl)anilide, and the background discoloration inhibitor is N,N'-di(m-tolyl)ethylene diamine.

11. A light-sensitive diazo composition as claimed in claim 7, wherein the light-sensitive diazonium compound is 4-morpholino-2,5-diisopropoxybenzenediazonium hexafluorophosphate; the coupling components are 2,2',4,4'-tetrahydroxy-3,3'-dimethylidiphenyl sulfide, 2,2',4,4'-tetrahydroxy-5,5'-dichlorodiphenyl sulfide, and 2-hydroxy-3-naphthoic acid-(3'-acetyl)anilide; and the background discoloration inhibitor is N,N'-di(p-tolyl)ethylene diamine.

12. A light-sensitive diazo composition as claimed in claim 7, wherein the light-sensitive diazonium compound is 4-morpholino-2,5-diisopropoxybenzenediazonium hexafluorophosphate; the coupling components are 2,2',4,4'-tetrahydroxy-3,3'-dimethylidiphenyl sulfide, 2,2',4,4'-tetrahydroxy-5,5'-dichlorodiphenyl sulfide, and 2-hydroxy-3-naphthoic acid-(3'-acetyl)anilide; and the background discoloration inhibitor is 1,3-di(p-tolyl)-2-phenyl-

ylimidazolidine.

13. A light-sensitive diazo composition as claimed in claim 7, wherein the light-sensitive diazonium compound is 4-morpholino-2,5-diisopropoxybenzenediazonium hexafluorophosphate; the coupling components are 2,2',4,4'-tetrahydroxy-3,3'-dimethylidiphenyl sulfide, 2,2',4,4'-tetrahydroxy-5,5'-dichlorodiphenyl sulfide, and 2-hydroxy-3-naphthoic acid-(3'-acetyl)anilide; and the background discoloration inhibitor is 1,3-di(m-tolyl)-2-phenylimidazolidine.

14. A light-sensitive diazo composition as claimed in claim 7, wherein the light-sensitive diazonium compound is 4-morpholino-2,5-diisopropoxybenzenediazonium hexafluorophosphate; the coupling components are 2,2',4,4'-tetrahydroxy-3,3'-dimethylidiphenyl sulfide, 2,2',4,4'-tetrahydroxy-5,5'-dichlorodiphenyl sulfide, 2-hydroxy-3-naphthoic acid (3'-sulfonamide) anilide; and 2-hydroxy-3-naphthoic acid (3'[N-methyl]sulfonamido)anilide; and the background discoloration inhibitor is 1,2,3-triphenylimidazolidine.

15. A light-sensitive diazo composition as claimed in claim 7, wherein the light-sensitive diazonium compounds is 4-morpholino-2,5-diisopropoxybenzenediazonium hexafluorophosphate, the coupling components are 2,2',4,4'-tetrahydroxy-3,3'-dimethylidiphenyl sulfide and 2-hydroxy-3-naphthoic acid (3'-acetyl)anilide, and the background discoloration inhibitor is 1,2,3-triphenylimidazolidine.

16. A light-sensitive diazo composition as claimed in claim 7, wherein the light-sensitive diazonium compound is 4-morpholino-2,5-diisopropoxybenzenediazonium hexafluorophosphate, the coupling components are 2,2',4,4'-tetrahydroxy-3,3'-dimethyl sulfoxide and 2-hydroxy-3-naphthoic acid (3'-acetyl)anilide, and the background discoloration inhibitor is 1,2,3-triphenylimidazolidine.

17. A light-sensitive diazo composition as claimed in claim 7, wherein the light-sensitive diazonium compound is 4-morpholino-2,5-diisopropoxybenzenediazonium hexafluorophosphate, the coupling components are 2,2',4,4'-tetrahydroxy-3,3'-dimethyl-5,5'-dichlorodiphenyl sulfide and 2-hydroxy-3-naphthoic acid (3'-acetyl)anilide and the background discoloration inhibitor is 1,2,3-triphenylimidazolidine.

18. A light-sensitive diazo composition as claimed in claim 7, wherein the light-sensitive diazonium compound is 4-morpholino-2,5-disopropoxybenzenediazonium hexafluorophosphate, the coupling components are diresorcylic sulfide and 2-hydroxy-3-naphthoic acid (3'-acetyl)anilide, and the background discoloration inhibitor is 1,2,3-triphenylimidazolidine.

19. A light-sensitive diazo composition as claimed in claim 7, wherein the light sensitive diazonium compound is 4-morpholino-2,5-diisopropoxybenzenediazonium hexafluorophosphate, the coupling components are diresorcylic sulfide and 2-hydroxy-3-naphthoic acid (3'-acetyl)anilide, and the background discoloration inhibitor is 1,2,3-triphenylimidazolidine.

20. A light-sensitive diazo composition as claimed in claim 7, wherein the light-sensitive diazonium compound is 4-morpholino-2,5-diisopropoxybenzenediazpmoi, hexafluorophosphate, the coupling components are diresorcinol and 2-hydroxy-3-naphthoic acid(3'-acetyl) anilide, and the background discoloration inhibitor is 1,2,3-triphenylimidazolidine.

21. A light-sensitive diazo composition as claimed in claim 7, wherein the light-sensitive diazonium compound is 4-morpholino-2,5-dicyclopentyloxybenzenediazonium hexafluorophosphate, the coupling components are 2,2',4,4'-tetrahydroxy-3,3'-dimethyl-5,5'-dichlorodiphenyl sulfide and 2-hydroxy-3-naphthoic acid(3'-acetyl)lidel, and the background discoloration inhibitor is 1,2,3-triphenylimidazolidine.

22. -tetrahydroxy-light-sensitive diazo composition as claimed in claim 7, wherein the light-sensitive diazonium com-

ound is 4-morpholino-2,5-di(secondary-butoxy)benzene diazonium hexafluorophosphate, the coupling components are 2,2',4,4'-tetrahydroxy-3,3'-dimethyl 5,5'-dichlorodiphenyl sulfide and 2-hydroxy-3-naphthoic acid (3'-acetyl)anilide, and the background discoloration inhibitor is 1,2,3-triphenylimidazolidine.

23. A diazotype material comprising a support and a diazo layer coated on said support, said layer comprising the light-sensitive diazo composition claimed in claim 1.

10 24. A diazotype material as claimed in claim 23, wherein the support is selected from the class consisting of paper, cloth, transparentized paper, a cellulose ether film a cellulose ester film and a polyester film having a subcoat thereon of cellulose acetate butyrate.

15 25. A diazotype material comprising a cellulose diacetate film as a support and a diazo layer coated on said support, said layer comprising the light-sensitive diazo composition claimed in claim 8.

20 26. A diazotype material comprising a cellulose diacetate film as a support and a diazo layer coated on said support, said layer comprising the light-sensitive diazo composition claimed in claim 9.

25 27. A diazotype material comprising a cellulose diacetate film as a support and a diazo layer coated on said support, said layer comprising the light-sensitive diazo composition claimed in claim 10.

30 28. A diazotype material comprising a cellulose diacetate film as a support and a diazo layer coated on said support, said layer comprising the light-sensitive diazo composition claimed in claim 11.

35 29. A diazotype material comprising a cellulose diacetate film as a support and a diazo layer coated on said support, said layer comprising the light-sensitive diazo composition claimed in claim 12.

30 30. A diazotype material comprising a cellulose diacetate film as a support and diazo layer coated on said support, said layer comprising the light-sensitive diazo composition claimed in claim 13.

35 31. A diazotype material comprising a cellulose diacetate film as a support and a diazo layer coated on said support, said layer comprising the light-sensitive diazo composition claimed in claim 14.

40 32. A diazotype material comprising a cellulose diacetate film as a support and a diazo layer coated on said support, said layer comprising the light-sensitive diazo composition claimed in claim 15.

45 33. A diazotype material comprising a cellulose diacetate film as a support and a diazo layer coated on said support, said layer comprising the light-sensitive diazo composition claimed in claim 16.

50 34. A diazotype material comprising a cellulose diacetate film as a support and a diazo layer coated on said support, said layer comprising the light-sensitive diazo composition claimed in claim 17.

55 35. A diazotype material comprising a cellulose diacetate film as a support and a diazo layer coated on said support, said layer comprising the light-sensitive diazo composition claimed in claim 18.

60 36. A diazotype material comprising a cellulose diacetate film as a support and a diazo layer coated on said support, said layer comprising the light-sensitive diazo composition claimed in claim 19.

65 37. A diazotype material comprising a cellulose diacetate film as a support and a diazo layer coated on said support, said layer comprising the light-sensitive diazo composition claimed in claim 20.

70 38. A diazotype material comprising a cellulose diacetate film as a support and a diazo layer coated on said support, said layer comprising the light-sensitive diazo composition claimed in claim 21.

39. A diazotype material comprising a cellulose diacetate film as a support and a diazo layer coated on said support, said layer comprising the light-sensitive diazo composition claimed in claim 21.

\* \* \* \* \*

UNITED STATES PATENT OFFICE  
CERTIFICATE OF CORRECTION

Patent No. 3,619,191 Dated November 9, 1971

Inventor(s) Robert C. Desjarlais Page 1 of 9

It is certified that error appears in the above-identified patent and that said Letters Patent are hereby corrected as shown below:

In the Specification:

Column 1, line 75, "diazotypec" should read --diazotype--.

Column 3, line 48, "4-morpholine" should read  
--4-morpholino--.

Column 3, line 49, insert the following: --(isopropoxy)  
benzene-diazonium chloride--.

Column 4, line 7, "cenzene" should read --benzene--.

Column 4, line 70, after "acid," and before "2 hydroxy"  
insert --2 hydroxy-3 naphthoic anilide--.

Column 4, lines 71 and 72, delete "2 hydroxy-3 naphthoic-  
(4' chloro) anilide,".

Column 5, line 16, "1-(Benzen 4' sulfonic acid)" should  
read --1-(Benzene-4' sulphonic acid) --.

Column 5, line 19, delete "N,N'-diaryl-substituted" and  
insert therefor --in--.

Column 5, line 21, delete "diazotype" and insert therefor  
--general--.

Cont.

UNITED STATES PATENT OFFICE  
CERTIFICATE OF CORRECTION

Patent No. 3,619,191 Dated November 9, 1971  
Inventor(s) Robert C. Desjarlais Page 2 of 9

It is certified that error appears in the above-identified patent and that said Letters Patent are hereby corrected as shown below:

Column 5, line 56, delete "onto" and insert therefor  
--are--.

Column 6, line 44, after "as" and before ",4,4'", insert  
--2,2'--.

Column 6, line 45, before ",4,4'" (both occurrences)  
insert --2,2'--.

Column 6, line 46, "5,5" should read --5,5'--.

Column 6, line 47, before ",4,4'", insert --2,2'--.

Column 6, line 60, after "of" and before ",4,4'" insert  
--2,2'--.

Column 7, line 6, after "2,2',4,4'" and before "3,3'-",  
insert -- -tetrahydroxy- --.

Column 7, line 14, after "24" and before "then", insert  
--hours--.

Column 7, line 19, "22',4,4'-tetrahydroxy" should read  
--2,2',4,4'-tetrahydroxy--.

Column 7, line 21, after ";" and before "5.15," insert  
"Hydrogen--." Cont.

UNITED STATES PATENT OFFICE  
CERTIFICATE OF CORRECTION

Patent No. 3,619,191 Dated November 9, 1971  
Inventor(s) Robert C. Desjarlais Page 3 of 9

It is certified that error appears in the above-identified patent and that said Letters Patent are hereby corrected as shown below:

Column 7, line 23, after "2,2',4,4'" and before "5,5'",  
insert -- -tetrahydroxy- --.

Column 7, line 44, after "2,2',4,4'" and before "5,5'",  
insert -- -tetrahydroxy- --.

Column 7, line 53, after "2,2',4,4'" and before "3,3'",  
insert -- -tetrahydroxy- --.

Column 7, line 70, delete "5.55" and insert therefor  
--3.55--.

Column 12, line 39, insert --4.23%-- in the column under  
"Found"; and delete the number or numbers which appear in the  
column under "Theoretical" and insert therefor --4.10%--.

Column 12, line 73, "n" should read --m--.

Column 12, line 74, "trifluoromethyl)" should read  
--(trifluoromethyl)--.

Column 14, line 21, "ro" should read --or--.

Column 14, line 24, after "to" (first occurrence) and  
before "five", insert --about--.

Cont.

UNITED STATES PATENT OFFICE  
CERTIFICATE OF CORRECTION

Patent No. 3,619,191 Dated November 9, 1971  
Inventor(s) Robert C. Desjarlais Page 4 of 9

It is certified that error appears in the above-identified patent and that said Letters Patent are hereby corrected as shown below:

Column 16, line 58, "as" should read --was--.

Column 16, line 66, insert --11.63-- in the column under "Found"; and delete the number or numbers which appear in the column under "Theoretical" and insert therefor --11.66--.

Column 17, line 26, "N,N" should read --N,N'--.

Column 17, line 53, "Triphenylimidazolidene" should read --Triphenylimidazolidine--.

Column 18, line 29, "illustrated" should read --illustrate--.

Column 18, line 39, delete "g." which appears under the column entitled "AMOUNT".

Column 18, line 46, "2Hydroxy" should read --2-Hydroxy--.

Column 18, line 63, delete the word "imidazolidine".

Column 19, line 1, "5" should read --4--.

Column 19, line 4, "dimethylethylene" should read --diphenylethylene--.

Column 19, line 28, "0.6g." should read --0.6 cc.--.

Column 19, line 32, "(3'[N-" should read --(3'-[N- --.

Cont.

UNITED STATES PATENT OFFICE  
CERTIFICATE OF CORRECTION

Patent No. 3,619,191 Dated November 9, 1971  
Inventor(s) Robert C. Desjarlais Page 5 of 9

It is certified that error appears in the above-identified patent and that said Letters Patent are hereby corrected as shown below:

Column 19, line 34, "2,2"--" should read --2,2',4,4'--.

Column 19, line 36, "hexfluorophosphate" should read  
--hexafluorophosphate--.

Column 19, line 55, "0.6g." should read --0.3gm.--.

Column 19, line 58, "0.75g" should be relocated so that it appears under the column entitled "AMOUNT".

Column 19, line 70, "2,2',4,4'" should read --2,2',4,4'-tetrahydroxy--.

Column 19, line 71, "2,2',4,4'3,3'-dimethyl 5,5'-dichlorodiphenyl" should read --2,2',4,4'-tetrahydroxy-3,3'-dimethyl-5,5'-dichlorodiphenyl--.

In the Claims:

Claim 1, lines 3 and 4 (Column 20, lines 19 and 20), "[derived from a dialkoxy - substituted - p-phenylene diamine]" should be deleted.

Cont.

UNITED STATES PATENT OFFICE  
CERTIFICATE OF CORRECTION

Patent No. 3,619,191 Dated November 9, 1971  
Inventor(s) Robert C. Desjarlais Page 6 of 9

It is certified that error appears in the above-identified patent and that said Letters Patent are hereby corrected as shown below:

Claim 1, on the line on which the fourth structural formula begins (Column 20, line 54), insert --(3)-- on the left-hand edge of the column.

Claim 1, on the line on which the fifth structural formula begins (Column 20, line 59), insert --(4)-- on the left-hand edge of the column.

Claim 1, last line (Column 20, line 68), after "atoms" and before ".", insert the following: --or a group represented by Ar; and R is a methylene group or an aryl-substituted methylene group; and

D. an acidic stabilizer--.

Claim 2, lines 2 to 6 (Column 20, lines 70 to 74), "[derived from 4-morpholino-2,5-diisopropoxyaniline, 4-morpholino-2,5-di(tertiary butoxy) aniline; 4-morpholino-2,5-di(secondary butoxy) aniline; or 4-morpholino-2,5-dicyclo-pentoxyaniline]" should be deleted.

Claim 3, line 8 (Column 21, line 11), "1,2,3 triphenylimidazolidene" should read --1,2,3-triphenylimidazolidine--.

Cont.

UNITED STATES PATENT OFFICE  
CERTIFICATE OF CORRECTION

Patent No. 3,619,191 Dated November 9, 1971  
Inventor(s) Robert C. Desjarlais Page 7 of 9

It is certified that error appears in the above-identified patent and that said Letters Patent are hereby corrected as shown below:

Claim 3, line 9 (Column 21, line 12), "ylimidazolidene" should read --ylimidazolidine--, and "1,3-di(p-tolyl)" should read --1,3-di-(p-tolyl)--.

Claim 3, line 10 (Column 21, line 13), "methylimidazolidene" should read --methylimidazolidine--, and "1,2,3 triphenyl 4" should read --1,2,3-triphenyl-4--.

Claim 4, line 2 (Column 21, line 17), after "the" and before "compound" insert --coupling components for the diazonium--.

Claim 8, line 3 (Column 22, line 37), "2.5" should read --2,5--.

Claim 9, line 6 (Column 22, line 48), "tetrohydroxy" should read --tetrahydroxy--.

Claim 13, line 3 (Column 23, line 4), "4 morpholino" should read --4-morpholino--.

Claim 13, line 5 (Column 23, line 6), "2,2--" should read --2,2',4,4'-- --.

Cont.

UNITED STATES PATENT OFFICE  
CERTIFICATE OF CORRECTION

Patent No. 3,619,191 Dated November 9, 1971  
Inventor(s) Robert C. Desjarlais Page 8 of 9

It is certified that error appears in the above-identified patent and that said Letters Patent are hereby corrected as shown below:

Claim 13, last line (Column 23, line 10), "ylimidizolidine" should read --ylimidazolidine--.

Claim 14, line 7 (Column 23, line 17), "sulfonamide" should read "sulfonamido- --.

Claim 15, line 2 (Column 23, line 22), "compounds" should read --compound--.

Claim 17, line 4 (Column 23, line 39), "2,2',4', "should read --2,2',4,4'--.

Claim 17, last line (Column 23, line 43), "iclne" should read --idine--.

Claim 18, line 3 (Column 23, line 46), "disopropoxybenaene-diazonium" should read --diisopropoxybenzenediazonium --.

Claim 20, line 3 (Column 23, line 61), "diisopropoxybenzene diazpmoi" should read --diisopropoxybenzenediazonium--.

Claim 21, line 6 (Column 23, line 71), "lide" should read --anilide--.

Claim 22, line 1 (Column 23, line 74), delete "-tetrahydroxy-" and insert therefor --A--.

Cont.

UNITED STATES PATENT OFFICE  
CERTIFICATE OF CORRECTION

Patent No. 3,619,191 Dated November 9, 1971  
Inventor(s) Robert C. Desjarlais Page 9 of 9

It is certified that error appears in the above-identified patent and that said Letters Patent are hereby corrected as shown below:

Claim 22, line 5 (Column 24, line 3), "diemthyl" should read --dimethyl--.

Claim 31, line 2 (Column 24, line 40), "daizo" should read --diazo--.

Claim 39, last line (Column 24, line 74, "21" should read --22--.

Signed and Sealed this  
Eighth Day of March 1977

(SEAL)

Attest:

RUTH C. MASON  
Attesting Officer

C. MARSHALL DANN  
Commissioner of Patents and Trademarks